

Nov. 26, 1940.

F. R. KRAUSE

2,223,039

## METHOD FOR ELONGATING METAL BLANKS

Original Filed Feb. 19, 1937 5 Sheets-Sheet 1

Fig. 1.



Fig. 2.



WITNESSES

A. B. Wallace.

U. A. Peckham.

Frank R. Krause  
BY Brown, Critchlow & Flick  
his ATTORNEYS.

Nov. 26, 1940.

F. R. KRAUSE

2,223,039

METHOD FOR ELONGATING METAL BLANKS

Original Filed Feb. 19, 1937 5 Sheets-Sheet 2



INVENTOR.

WITNESSES

A. Wallace.

V. A. Puckham.

BY

Frank R. Krause  
Brown, Crittenden & Flick  
his ATTORNEYS.

Nov. 26, 1940.

F. R. KRAUSE

2,223,039

METHOD FOR ELONGATING METAL BLANKS

Original Filed Feb. 19, 1937 5 Sheets-Sheet 3

Fig. 4.



Fig. 5.



INVENTOR.

WITNESSES

A. B. Wallace.

V. A. Pickham.

Frank R. Krause  
BY Brown, Britallow & Hicks  
his ATTORNEYS.

Nov. 26, 1940.

F. R. KRAUSE

2,223,039

METHOD FOR ELONGATING METAL BLANKS

Original Filed Feb. 19, 1937 5 Sheets-Sheet 4



INVENTOR.

Frank R. Krause

BY Brown, Crittlow & Neely

his ATTORNEYS.

WITNESSES

A. B. Wallace.

V. A. Pickham.

Nov. 26, 1940.

F. R. KRAUSE

2,223,039

## METHOD FOR ELONGATING METAL BLANKS

Original Filed Feb. 19, 1937 5 Sheets-Sheet 5



**WITNESSES**

A. B. Wallace.

V. A. Peckham

INVENTOR.

BY Frank P. Krause  
Brown, Critchlow & Flick  
his ATTORNEYS

## UNITED STATES PATENT OFFICE

2,223,039

## METHOD FOR ELONGATING METAL BLANKS

Frank R. Krause, Ellwood City, Pa.

Original application February 19, 1937, Serial No. 126,633. Divided and this application October 22, 1938, Serial No. 236,457.

13 Claims. (Cl. 80—60)

This invention relates to a method for reducing and elongating metal blanks.

In metal rolling, as generally practiced today, it generally requires a series of substantially full length passes through a rolling mill to reduce a blank to the desired thickness or gauge, the reduction in any one pass being only a fraction of the total reduction. The reduction that can be made in any one pass is limited by the tendency of the rolls to slip against the blank if too great a draft is attempted to be taken. In fact, if the draft is too great the blank will not even enter the roll pass. In rolling thin sections such as strip, the amount of draft is also limited by the tendency of the metal to tear transversely at the center of the roll pass due to the friction force between the rolls and blank having a greater velocity in the direction of rolling at the pass center than at the first zone of contact of rolls and blank. Furthermore, the blank is rolled in one continuous operation from its front end to its rear end in each pass, whereby the rolls constantly roll against the thickest portion of the blank with a uniform draft which requires a great deal of power. When a single mill stand is used, for each successive reduction the entire blank must pass through the mill which is thus subjected to considerable strain and wear in reducing each blank to the gauge desired.

It is among the objects of this invention to provide a method for reducing metal blanks in which any desired reduction can be obtained in passing a blank through a single mill stand only once, in which the draft is not limited to the coefficient of friction for the blank and reducing means in which the character of the metal of the blank is improved, in which spreading of the blank is reduced to a minimum, and in which the life and capacity of the mill is increased.

In accordance with this invention a metal blank is reduced to any desired gauge or thickness by passing it once only through a mill having reducing means, such as a roll or rolls, which are caused to periodically move toward the front or entering end of the blank. During each of these working strokes the reducing means also first move toward the axis or central plane of the blank and then in paths parallel to that axis, whereby the unreduced portion of the blank is connected by a tapered or wedge-shaped portion to a flat reduced portion. The movement of reducing rolls is brought about by relative reciprocal movement between the blank and a pair of track surfaces that back up and engage the rolls. The shape of these tracks determines the amount

of reduction. The unrolled portion of the blank and the track surfaces are held against movement in the same direction during the reducing steps so that the rolls have a definite drawing action on the blank as well as a pressing action. The rotation of the rolls is controlled principally by their frictional engagement with the track surfaces and blank, and the axes of the rolls are therefore free to accommodate themselves to the relative speeds of the tracks and blank. That is, the rolls float by which is meant the rolls are not restricted by mechanical means in their movement along the blank and therefore can follow the elongation of the blank as the metal is displaced. During the return strokes of the rolls between working strokes, unrolled increments of the blank are successively brought into position for reduction by the rolls. It will therefore be understood that in the practice of my invention a blank is reduced to desired gauge in passing once only through a single mill stand by a step-by-step feed.

Apparatus suitable for practicing my invention is illustrated in the accompanying drawings in which Fig. 1 is a plan view, partly in section, of a rolling mill and blank-clamping and pushing apparatus; Fig. 2 is a central vertical section thereof, except that the upper roll is shown in elevation; Fig. 3 is an enlarged view of the delivery end of the mill, half of it being shown in section; Fig. 4 is a plan view of apparatus for actuating the mill; Fig. 5 is a central vertical section thereof; Fig. 6 is a plan view of apparatus for feeding blanks to the mill; Fig. 7 is a central vertical section thereof; Fig. 8 is an enlarged fragmentary view of Fig. 2; Fig. 9 is an end view of the blank-clamping apparatus taken on the line IX—IX of Fig. 2; Fig. 10 is a vertical section of the blank pusher taken on the line X—X of Fig. 2; and Fig. 11 is a view showing diagrammatically the relative positions of tracks and rolls at different stages of a working stroke, the tracks being of a modified form.

Referring to the drawings, a track housing 1, provided with an opening 2 extending from end to end thereof and having parallel horizontal and vertical side walls, is slidably mounted on a bed-plate 3, Figs. 1, 2 and 3. Rigidly secured to the sides of the track housing and projecting forwardly therefrom are a pair of rods 4 connected at their front ends by a crosshead 6 slidably mounted on an extension of the bed-plate, Figs. 4 and 5. Pivotedly mounted on the opposite ends of the crosshead are crank arms 7 which are actuated by large heavy gears 8 mounted on the

opposite ends of a crank shaft 10 journaled in the bed-plate. The gears are rotated by pinions 9 turned by a drive shaft 11 likewise journaled in the bed-plate and driven by any suitable source 5 of power.

Removably mounted in the top and bottom walls of housing opening 2 is a pair of tempered steel track plates 12 between which a roll carriage 13 is slidably disposed for movement longitudinally of the opening. The carriage is guided 10 in a straight line by a forward extension terminating in an inverted channel 14 slidably mounted on a rail 15 projecting from the front of the track housing. Journaled in bearing blocks 16 (Figs. 3 and 8) slidably mounted in vertical recesses in the side walls of the roll carriage 15 is a pair of superimposed reducing rolls 17 which are biased apart by coil springs 18 compressed between the bearing blocks, Fig. 3.

20 To permit the size of the roll pass to be varied for reducing blanks of different thicknesses to different gauges, the upper wall of opening 2 is formed by a cap 19 slidable vertically in the upper portion of the housing. This cap is biased upwardly by a coil spring 20 compressed between the top of a recess 21 in the center of the cap and the head of a bolt 22 suspended from a cross bar 23 affixed to the top of the housing. The cap is adjusted downwardly by wedges 24 between the cap and laterally spaced ribs 26 integral with the housing, Fig. 3. The wedges are spaced from the cap by segmental shoes 27 which facilitate transverse rocking of the cap when only one wedge is adjusted. To permit the wedges to be 30 moved in and out, their rear ends are provided with threaded rods 28 slidable in brackets 29 secured to the back of the housing, the rods being provided with adjusting nuts 31, Figs. 1 and 2.

It is a feature of this invention that the track 40 plates are so formed that, as the track housing is moved forward by the cranks during each working stroke, the track plates carried by it roll the rolls forward against the stationary blank 32 toward its front end and simultaneously toward each other whereby, by a combined rolling, sinking and drawing operation, they reduce and elongate the blank. During the latter part of the working stroke the rolls travel parallel to the central longitudinal plane of the blank to form 50 flat reduced material, metal strip being shown in the drawings for the purpose of illustration. As the rolls float; that is, as the axes of the rolls are free to accommodate themselves to the relative speeds of the tracks and blank, the rolls are carried forward by the elongating blank.

Accordingly, as shown in Figs. 2 and 8, the tracks are provided adjacent their rear ends with parallel areas 33 merging into areas 34 inclined away from each other toward the front of the track housing. Consequently, as the track housing moves forward from a position in which the rolls loosely engage an unreduced increment of the blank a portion of which has already been 60 reduced during preceding working strokes of the mill, the inclined areas of the tracks move into frictional engagement with the rolls and force them tightly against the blank. Continued movement of the tracks causes these rolls to roll forward and inwardly at the same time. This reduces the previously unrolled increment to tapered form and further reduces the blank's previously tapered portion, the thinner end of which is thus reduced to thin flat strip by the rolls when 70 the parallel areas of the tracks reach them and

move them in parallel paths as shown in Figs. 2 and 8.

The rolls are parallel to each other until the diverging rear ends of the track plates reach them, whereupon they are permitted to spread 5 apart and become released from the strip. While the track housing is continuing to move forward a short distance before its movement is reversed, the roll carriage is pushed forward with it. This is preferably done by a fluid pressure cylinder 36 10 mounted on the rear end of the bed-plate with its piston rod 37 connected to the carriage, as shown in Fig. 2. Thus, when the track plates start their return stroke they cause the rolls to start rolling back from a point on the strip in 15 front of the point at which the rolls were released from the strip. Consequently, the diverging areas at the front of the track plates reach the rolls before the latter reach the tapered portion of the strip so that the rolls will not roll that 20 tapered portion during their return stroke.

The return of the roll carriage is accomplished more smoothly if chains 39 are secured to the rear end of the bed-plate and trained around sprockets 40 loosely mounted on the ends of 25 the rolls. The opposite or front ends of the chains are connected to the rear of the track housing by coil springs 41 that allow the roll carriage to be pushed forward with the track housing by piston rod 37 after the rolls reach the 30 diverging rear ends of the tracks. On the return stroke of the housing the chains and sprockets insure the smooth return movement of the rolls, and near the end of the return stroke springs 41 expand and thereby restore the rolls to their original starting position relative to the tracks. At the conclusion of the return stroke the fluid under pressure is reversed to the front end of the cylinder, by any well known means (not shown), to hold the roll carriage stationary at the start of 40 the next working stroke until the rolls are brought into firm frictional engagement with the blank and tracks by the latter.

The drawings described thus far show the inclined or diverging areas of the tracks flat lengthwise. This shape of track is satisfactory when thin blanks, such as strip substantially not over  $\frac{1}{8}$  inch thick, are being reduced, because the necessary reduction can be made with the desired short working stroke of the mill without increasing the degree of inclination of track areas 34 to the point at which slippage of the rolls against the blank would occur. To be safe, the inclination should probably not exceed  $5^\circ$ . With thicker blanks, where the percentage of reduction is likely 50 to be greater than in the case of thin blanks, roll slippage is prevented without increasing the length of the working stroke or track by forming each inclined area 34 of a track plate in the shape of a reverse curve with its front end nearly horizontal (preferably  $1\frac{1}{2}^\circ$  to  $2^\circ$ ) and its central portion more steeply inclined to the horizontal, as 60 shown in Fig. 11. The latter inclination can be considerably greater than  $5^\circ$ .

As just indicated, the principal reason for this 65 shape of track is to prevent the rolls from slipping on the tracks or blank during the short working strokes that are desirable from the standpoint of rapid operation. The likelihood of 70 roll slippage on the blank is greatest when they first move into contact with the blank, and also when they approach the smaller end of the tapered portion of the blank where they come into contact with the parallel areas of the track. With 75

tracks of the shape just referred to, the draft is gradually increased during the beginning and gradually decreased during the ending of the working stroke of the mill so that there will be no roll slippage at those times. The heaviest draft is taken near the thicker end of the blank's tapered portion which is strong enough to withstand it, and the draft is gradually and materially decreased at the thinner end to prevent tearing the blank apart at its weak section.

With track plates of either shape, each successive draft starts at zero at the surface of an unreduced increment and gradually increases to its maximum amount. This gradual increase of the draft with its accompanying reduction orients the crystals in the metal before subjecting them to more severe elongations, and thereby improves the character of the metal. This improved portion of the metal is not affected adversely during the next working stroke of the mill when it is subjected to the maximum draft, but is still further improved because this maximum draft as effected in my mill causes only gradually increasing elongation of the stock and very little spreading thereof. In prior rolling practice in which rolls roll a blank from front to rear and continuously against the portion of a blank having the greatest thickness, the start of the draft at any given point along the stock is sudden instead of gradual and the crystals may therefore be caused to fracture when elongated under heavy drafts. The small amount of spreading in my mill is shown by samples of steel rolled cold therein in which elongations of as much as 30 to 1 were obtained in a single passage through the mill with a spreading of 25 per cent of that obtained with like pieces of steel rolled in a two-high mill giving elongation of only 16 to 1. The rolls used in both mills were all of the same diameter. The steel strip rolled in my mill was sound and pliable with smooth edges, but the strip rolled in the two-high mill with a 16 to 1 elongation was hard and had rough and torn edges.

The shape of the reverse curve tracks and the outline of a blank rolled between them is shown roughly in the diagram of Fig. 11 where the relation of the different members to one another when in three different positions is also illustrated. The full lines indicate the shape of a blank in the process of being reduced, and also the positions of the track plates and rolls during the beginning of a working stroke after the blank has first been advanced a step to subject an unrolled increment A-B to the action of the rolls. As the tracks continue to advance to the position indicated by broken lines they roll the rolls forwardly and inwardly into their broken line position wherein increment A-B and the adjoining portion of the tapered section of the blank are reduced an amount also shown by broken lines. It will be seen that at this stage the increment A-B has been reduced but slightly, the reduction increasing as the front of the increment is approached. On the other hand, the previously reduced portion of the blank near line C is reduced materially during this particular working stroke, due to the steeply inclined area of the track plates engaging the rolls. As the tracks continue to advance to the dotted line position in which their parallel areas reach the rolls, also dotted, the blank is reduced to the shape indicated by both broken and dotted lines. The portion C-D is reduced materially, but as line D is approached the draft starts to dimin-

ish, and by the time the rear ends of the tracks reach the rolls another portion of flat reduced material has been added to the preceding completely reduced portion.

With this type of mill in which rolls roll successive increments of a blank toward its front or entering end while the rolls bodily approach each other, blanks can be reduced in a single pass through the mill an amount heretofore thought impossible, because no greater draft is necessary for making a large reduction than for making a small one. This is because the amount of reduction does not depend upon the draft, which is governed by the distance the blank is fed forward each time, but upon the shape of the tracks and the length of the mill's working stroke. It will be understood that "draft" refers to the thickness of the metal removed by the rolls each time they roll along the blank, while "reduction" refers to the difference between the thickness of the unrolled blank and the finished rolled portion thereof.

The track plates can be so shaped that large reductions can be made with short working strokes, because roll slippage is prevented by the shape of the ends of the inclined areas of the track plates. Also, the rolls float between the track plates and are not turned through their axes but at their peripheries, so that the apex of the contact angle F of each roll is at the point of engagement of the roll with the track. Consequently, the contact angle is smaller for any given draft than for a like draft in a mill in which the apex of the contact angle is at the axis of a roll. The smaller the contact angle the less the tension stress on the blank from a force exerted longitudinally thereof toward the rolls, and also the less the likelihood of slippage of the rolls against the blank. The two forces acting in opposite directions to turn each roll are exerted at the periphery of the roll at its points of contact with the blank and adjoining track, whereby the leverage used in turning the roll is about twice as great as when one of those forces is exerted at the axis of the roll, and the roll offers about half as much resistance to turning. This factor also contributes to reduction in tension stress on the blank and in the likelihood of slippage of rolls against blank and tracks.

Another factor that differentiates this mill from those known heretofore is that the metal under rolling pressure is distributed on both sides of the vertical center line of the rolls, instead of all on one side of that line. This particular area of metal is indicated by the character E in Fig. 11. As the metal must therefore be displaced on both sides of this center line it must naturally flow in opposite directions therefrom, as indicated by the arrows, whereby the metal in the pass is under tension as well as compression as it is being displaced and therefore spreads less than in any other rolling practice in use today. As the flow of metal in this case is due to a combination of tension and compression forces, the metal pressure or separating force exerted on the rolls is less than it would be if compression forces alone were relied upon to reduce the blank. An advantage flowing from this is that the blank and the mill are subjected to less strain than heretofore and the capacity and life of the mill are therefore increased. Distribution of metal on both sides of the center line of the rolls also prevents the metal from backing away bodily from the center of the pass as there has previously been a tendency to do in

5 mills wherein a single wedge-like body of metal is held in contact with the rolls only by friction force that tends to pull it into the pass only by surface action on the metal. The metal just entering the roll pass and in contact with the rolls does not move noticeably relative to the surface of the rolls in going through the pass, and therefore this "no-slip" area of metal carries or floats the rolls along with it while they are rotating.

10 This results in considerably less rotation of the rolls for a given amount of linear travel than in any other mill of which I know.

15 As indicated before, while the track housing is making its return stroke, i. e., returning to its starting point during each cycle, and while the rolls are released from the blank, the blank is fed or advanced a step to subject the next succeeding unrolled or unreduced increment thereof to the action of the rolls.

20 A desirable feeding apparatus for this purpose is illustrated in the drawings wherein a slide 42 is slidable toward and away from the mill in a longitudinally extending recess 43 in a table 44. As shown in Fig. 10, the opposite side walls of the recess are provided with a pair of inwardly projecting ribs 45 below which extend flanges 46 projecting laterally from the bottom of the slide to hold it in the recess. The rear end of the blank is clamped to the slide by means of 25 a bar 47 bolted to the top of the slide. The slide is moved toward the mill by a piston rod 48 connected to a piston 49 disposed in a cylinder 51 located at the rear of table 44, Figs. 6 and 7. The piston is constantly biased toward 30 the mill by fluid pressure behind it in the cylinder, but its forward movement is obstructed at predetermined intervals by fluid in the cylinder in front of the piston. That is, a predetermined volume of fluid in front of the piston is released 35 from the cylinder at periodic intervals, the piston being forced ahead by the pressure behind it each time this occurs.

40 Suitable automatic means for releasing fluid from the front of the cylinder is shown in Fig. 7. 45 A pipe 52 extends from the front end of the cylinder down through a housing 53 to a drain or sump. The pipe is provided within the housing with a shut-off valve 54 which is actuated by a lever 56 biased forwardly to closed position 50 against a pin stop 57 by a coil spring 58. Slidably mounted in the housing above this valve is a rod 59 the front end of which is connected to the bottom of the track housing, as shown in Fig. 2. Within the valve housing a depending 55 dog 61 is pivoted to the rod and biased forwardly against a pin stop 62 by a coil spring 63. When the track housing starts its return stroke from the position shown in Fig. 2, the rod is slid backwardly through the housing to cause dog 61 to engage the valve lever and swing it backwardly to open the valve. As the valve is opened fluid escapes from the front of the cylinder and fluid pressure behind the piston moves it forward to feed the blank ahead a step. As the dog continues to move backwardly it slides off the end of the valve lever which is immediately jerked forward to closed position by coil spring 63. This closing of the valve stops the piston and blank feed. When the dog is moved forwardly 65 by the advancing track housing it passes over the end of the lever and then is pulled forward against stop 62 by spring 63. The volume of fluid that is permitted to escape from the front of the cylinder each time valve 54 is opened determines the amount of feed of piston and blank.

70 and this volume is controlled by an adjustable valve 64 in the pipe above the shut-off valve.

75 At periodic intervals, i. e., for the duration of each working stroke of the mill, the blank is held in fixed position by an automatic clamp shown most clearly in Fig. 9. Due to the fact that the unrolled portion of the blank is thus held in fixed position during rolling, the rolls exert a drawing action on the blank. The clamp includes a support 66 provided at one side with a bracket 67 in which is pivotally mounted one end of an arm 68 that extends across the top of the support with its opposite end connected by a depending link 69 to a piston 71 disposed in a hydraulic cylinder 72. Mounted on support 15 66 is a table 73 that supports the blank above which is a clamping head 74 connected to arm 68 by which it is forced down to clamp the blank against table 73 when the arm is drawn down by piston 71. To permit the clamping head to 20 accommodate itself to blanks of different thicknesses, it is preferably made self-aligning by providing its upper surface with a concave recess in which is seated a convex bearing 76 projecting from the bottom of the arm. The clamping 25 head is held against this bearing by a bolt 77 extending up through an oversized opening in the head and biased upwardly by a coil spring 78 encircling it in a recess in the top of the arm. Fluid pressure is automatically supplied to the 30 hydraulic cylinder and released therefrom by any well-known automatic control which may be actuated by the reciprocating track housing if desired.

35 To summarize the operation of the mill described herein, a blank 32 is held at its rear end in pusher slide 42 which at that time is at the rear end of table 44. With the blank clamped in fixed position by clamping head 74 with its front end in the roll pass, drive shaft 11 is 40 rotated which, by means of cranks 7 and rods 4, moves track housing 1 forward whereby rolls 17 taper the end of the blank before running off the end of it. During the return or backward stroke of the mill the clamp releases the blank which is 45 then fed forward an increment by the slide which is pushed forward by piston 49 in the manner described above. As soon as movement of the piston is arrested by the closing of valve 54, the blank is again clamped in place by head 50 54, and the rolls start forward again and taper an unreduced increment of the blank and further reduce the previously tapered end thereof. This tapering alone continues until a sufficient length of the blank extends far enough through 55 the roll pass to be engaged by the rolls throughout their working stroke, whereupon the foremost portion of the blank is engaged by the rolls while they are moving parallel to each other between track areas 33 and a flat reduced portion 60 of the blank of uniform gauge is produced. The blank continues to be fed ahead step by step, and after each feeding step a new increment of the blank is tapered by the mill rolls and the front end of the previously tapered portion is 65 flattened and added to the next preceding finished portion of the blank. In the case of strip, it is wound up into a coil 79 (Fig. 5) on a suitable tension reel (not shown).

70 This invention is particularly applicable to 70 the cold reducing of metal blanks, and some of the advantages mentioned, such as improvement of the grain structure of the blank and substantially unlimited reduction in one pass through the mill, relate to cold working. Nevertheless it 75

will be understood that the invention can likewise be practiced to advantage in the hot reducing of metal blanks.

Although the invention has been described as 5 contemplating holding the blank stationary while the mill is reciprocated to reduce it, it will be understood that the mill can be stationary and the blank reciprocated in it as it is fed through the mill.

10 According to the provisions of the Patent Statutes, I have explained the principle and mode of operation of my invention and have illustrated and described what I now consider to represent its best embodiment. However, I desire to have 15 it understood that, within the scope of the appended claims, the invention may be practiced otherwise than as specifically illustrated and described.

This application is a division of my copending application Serial No. 126,633, filed February 19, 1937, now Patent No. 2,161,064.

I claim:

1. The step-by-step method of rolling a metal blank toward its front end periodically by successive increments, in which rotation of a roll is effected and controlled only by opposing forces acting on opposite sides of the roll at its periphery.

2. The method of reducing a metal blank step 30 by step in successive increments by periodically rolling a roll toward the front end of the blank by means of a track member frictionally engaging the periphery of the roll, comprising leaving the roll free to accommodate itself to the relative speeds of said track member and blank.

3. The method of reducing a blank between a 35 pair of backed-up rolls, comprising effecting relative reciprocal movement between said rolls and blank longitudinally of the blank to cause the rolls to periodically roll toward the front end of the blank, the axes of the rolls being free to accommodate themselves to the relative speeds of the blank and roll backing-up means, moving the rolls first toward each other and then substantially parallel to each other as they approach the front of the blank to reduce and elongate a portion thereof, and periodically subjecting successive unrolled increments of the blank to the action of said rolls.

4. The method of reducing a metal blank between a pair of rolls, comprising simultaneously rolling the rolls toward the front end first of said blank and toward and then substantially parallel to each other to reduce and elongate a portion of the blank, the rotation of the rolls being controlled principally by their frictional engagement with the blank and force-applying means engaging the periphery of the rolls, advancing the blank a step, and repeating said rolling starting with an unreduced increment of the blank.

5. The method of reducing a metal blank between a pair of rolls, comprising rolling a portion thereof simultaneously toward the entering end of the blank and the central plane thereof to taper said portion while holding the unrolled portion of the blank against movement in the direction of rolling, continuing the rolling parallel to said plane to produce a flat reduced portion, and periodically repeating the entire rolling operation starting with a succeeding unrolled increment of the blank each time.

6. The method of reducing a metal blank between a pair of rolls, comprising simultaneously 75 rolling the rolls toward the front end of said

blank and toward each other to reduce and elongate a portion of the blank, continuing the rolling with the rolls moving in substantially parallel paths, said rolling movement of the rolls being caused solely by opposing forces acting only 5 at the periphery of said rolls, and periodically advancing successive unrolled increments of said blank for reduction by said rolls.

7. The method of reducing a metal blank between a pair of back-up rolls, comprising simultaneously rolling the rolls toward the front end of said blank and toward each other to reduce and elongate a portion of the blank, continuing the rolling with the rolls moving in substantially parallel paths, the rolls being free to accommodate themselves to the relative speeds of the blank and roll backing-up means, releasing the rolls from said blank and moving them toward the rear end of the blank, advancing the blank an increment, repeating said rolling starting with 20 an unreduced increment of the blank, and holding the unrolled portion of the blank in substantially fixed position during each blank-reducing step.

8. The method of reducing a metal blank, comprising simultaneously rolling a pair of rolls toward the front end of said blank and gradually toward each other, continuing the rolling with the rolls approaching each other more rapidly followed by a more gradual approach, advancing 30 the blank a step, and repeating said rolling starting with an unreduced increment of the blank.

9. The method of reducing a metal blank between a pair of rolls, comprising rolling a portion thereof simultaneously toward the entering end 35 of the blank and the central plane thereof to taper said portion, continuing the rolling parallel to said plane to produce a flat reduced strip, returning the rolls to their original position, advancing the blank a step, repeating the entire 40 rolling operation starting with an unrolled increment of the blank, holding the unrolled portion of the blank in substantially fixed position during each blank-reducing step, said increment being tapered and said previously tapered portion 45 being further reduced with its thinner end reduced to flat form during said second rolling operation, and repeating the entire cycle of operation until substantially the entire blank is rolled down to flat reduced form.

10. The step-by-step method of reducing a metal blank in successive increments, comprising effecting relative reciprocal movement between said blank and blank-reducing means longitudinally of the blank to cause said means to periodically move toward the front end of the blank, moving said means first toward and then substantially parallel to the axis of the blank as it approaches the front of the blank to reduce and elongate a portion thereof, and leaving said 55 means free to accommodate itself to the elongation of the blank.

11. The step-by-step method of reducing a metal blank in successive increments, comprising 65 effective relative reciprocal movement between said blank and blank-reducing means longitudinally of the blank to cause said means to periodically move toward the front end of the blank, moving said means first toward and then substantially parallel to the axis of the blank as it approaches the front of the blank to reduce and elongate a portion thereof, leaving said means free to accommodate itself to the elongation of the blank, and holding the unrolled portion of 70 75

the blank against movement in the direction of elongation during each blank-reducing step.

12. The method of reducing a metal blank step by step in successive increments, comprising periodically rolling a freely floating roll toward the front end of the blank and simultaneously first toward and then substantially parallel to the axis of the blank.

13. The method of reducing a metal blank, comprising simultaneously rolling a pair of rolls

toward the front end of said blank and toward each other in planes intersecting the axis of the blank at an angle of approximately  $2^{\circ}$ , continuing the rolling with the rolls approaching each other in planes intersecting said axis at an angle substantially greater than  $5^{\circ}$  followed by a more gradual approach, advancing the blank a step, and repeating said rolling starting with an un-reduced increment of the blank.

FRANK R. KRAUSE. 10